

J. H. REID.

PROCESS FOR MAKING CARBID.  
APPLICATION FILED SEPT. 21, 1917.

1,396,058.

Patented Nov. 8, 1921.

FIG. 1.



FIG. 2.



FIG. 3.



Witnesses

Lloyd R. Cornwall.

Inventor  
James Harry Reid  
By May Totten & Parrot  
Attorneys

# UNITED STATES PATENT OFFICE.

JAMES HENRY REID, OF PITTSBURGH, PENNSYLVANIA, ASSIGNOR TO INTERNATIONAL NITROGEN COMPANY, A CORPORATION OF DELAWARE.

## PROCESS FOR MAKING CARBID.

1,396,058.

Specification of Letters Patent.

Patented Nov. 8, 1921.

Application filed September 21, 1917. Serial No. 192,487.

*To all whom it may concern:*

Be it known that I, JAMES HENRY REID, a citizen of the United States, and resident of Pittsburgh, in the county of Allegheny and State of Pennsylvania, have invented a new and useful Improvement in Processes for Making Carbid; and I do hereby declare the following to be a full, clear, and exact description thereof.

10 This invention relates to a process of making carbid such, for example, as calcium carbid. It is to be understood, however, that the invention comprehends both metal and non-metal carbids.

15 The invention has for its object, among others, the production of carbids by the action of heat in such manner that a more perfect conversion may be obtained with less heat, in shorter time, and the expenditure of less energy, such as electrical energy, than has been possible in the processes employed heretofore.

Moreover, the process is so designed that the product is removed from the zone of action as fast as it is formed, so that only sufficient energy is consumed to produce the carbid which is not subsequently subjected to over-heating, nor is it retained within the action of the heat zone for a longer time than is necessary to produce and discharge the same.

A further object is the production of a substantially non-contaminated product.

Further, the proportion of carbon in the material to be converted may be just sufficient to form a carbid from the desired oxid.

The material from which the carbid is produced comprises a cemented mixture of an oxid and carbon. This oxid and carbon mixture, for example, may be a lime-carbon coke material, such as produced from the carbonization or decomposition by heat of a mixture of bituminous coal and lime. The calcium oxid is saturated with hydrocarbons from the decomposition of the coal and carbon is deposited evenly throughout the lime by decomposition of the hydrocarbons. The carbon, so deposited, is rigidly attached to and is not separable from the oxid by vibration or such other physical action as may be encountered in an electrical furnace.

Calcium oxid, for example, when sub-

jected to this process contains rigidly attached carbon and forms a material from which a carbid may be produced of more perfect character in less time and with less expenditure of energy, and produces a more perfect conversion and a purer product than has been procured by processes heretofore.

My process comprises feeding aggregates of oxid and carbon to a heat reaction zone, induced and maintained by the passage of electricity through the material between electrodes, where it is converted into the desired product, and discharged therefrom by gravity or other means. In the operation of my process it is found desirable to permit the discharge of molten carbid as rapidly as possible, meanwhile preventing the passage of unconverted solid material. This may be accomplished by means of a barrier or hearth placed immediately below the zone of extreme heat but sufficiently removed from the electrodes so that it does not short-circuit the furnace by causing the electric current to pass directly from the electrode through the hearth. The accompanying drawing shows a type of construction that may be used in the operation of my process.

As an example of the process and the manner in which the same is carried out, the making of calcium carbid from lime-carbon coke by the action of heat induced by electricity will be taken; reference being directed to the accompanying drawings, in which,

Figure 1 is a longitudinal vertical section of an electric furnace;

Fig. 2 is a sectional view on the lines 2—2;

Fig. 3 is a top plan view thereof.

Similar letters of reference indicate corresponding parts in the various views.

Referring to the drawings, the numeral 1, indicates an electric furnace provided with the feed receptacle 2, into which projects the electrodes 3 and 4, provided with the electrical contact attachments 5 and 6, which electrodes 3 and 4, are so arranged as to deliver electricity to and from each other through the material 7, to be converted into carbid, and the hearth 8, so situated as to radiate and supply heat to and through the material from which the carbid is made, which hearth 8, also provides

means for obstructing the passage of material unconverted into carbid, until it is converted, and a means for separating the molten carbid formed, from the unconverted ingredients and discharging it in a molten condition.

The carbid falling from the hearth 8, accumulates at 10, whence it may be drawn or raked out from time to time.

- 10 The electrodes 3 and 4 composed of an electrically conductive carbon, such as graphitic carbon, are provided with rest or guide sections 11 and 12 suitably supported in the walls of the furnace. These supports 15 are designed to direct the electrodes toward the hearth 8 in such manner that they will coact and coöperate with the hearth to concentrate the necessary amount of heat upon and through the ingredients to be transformed 20 into carbid. Thus as the carbid is formed it is discharged from the heat zone in a molten state by gravity. This avoids over-heating to a point of decomposition of the carbid or the production of other substances which would be formed through 25 continued over-heating of the carbid which decomposition or formation of other substances would contaminate the desired product so as to be more or less detrimental to 30 the production of pure acetylene or nitrogen containing products of a uniform nature when the carbid is acted upon by water or nitrogen.

The floor 13 of the furnace upon which 35 the carbid accumulates is of suitable material inert to the carbid produced to prevent contamination of the product and the product may be removed by withdrawing or raking the same therefrom through either 40 outlet 14 or 15.

The heat in the furnace is produced by the action of electricity passing through the resistant material 7 between the electrodes 3 and 4.

- 45 In making calcium carbid, an intimate or pulverized mixture of a calcium oxy-compound, such as calcium oxide with bituminous coal, is heated to form a homogeneous mixture of oxid and carbon or, in other words, 50 what I term lime-carbon coke. The hydrocarbons evolved from the bituminous coal initially saturate each particle of the lime and are finally disassociated by the action of heat, leaving a lime to and within which 55 the carbon is rigidly cemented. This product is more uniformly resistant to the passage of a current of electricity than a loose mixture of calcium oxide and coke as ordinarily employed. The lime and carbon in 60 this cemented mixture cannot be separated from each other by electrical vibration which accentuates the difference in specific gravity between them. This separation is a serious defect in the processes now employed.

The homogeneous mixture of lime-carbon coke is then broken into small pieces and fed into an electric furnace, as shown in the accompanying drawings at the numeral 7, between the electrodes 3 and 4.

A current of electricity is then passed through the electrodes 3 and 4, by means of the contacts 5 and 6, communicating with a source of electricity, not shown.

As the electricity passes through the terminals of the electrodes and through the lower portions of the mass of oxid carbon coke, such as lime-carbon coke, for example, the resistance to the passage of the current generates a steadily increasing heat which 75 soon reaches a point at which the material is converted into carbid. The heat of formation still further augments the formation of the carbid and also facilitates the flow and discharge of the carbid from the heat 80 zone of formation, thus making way for a fresh supply of material to the heat zone by gravity or other means. The reaction is further augmented by the combustion of the carbon monoxid liberated in the reaction.

The molten calcium carbid formed, falls from the heated hearth 8 and accumulates on the floor 13 of the furnace, as shown at 10, from which place it may be withdrawn 95 or secured from time to time as desired.

The dominant principle governing this furnace is resistance. It does not function as an arc furnace. The oxid carbon coke is properly proportioned, mechanically and chemically mixed, and physically cemented into a solid homogeneous mass. The chief function of the furnace is to heat the oxid-carbon coke by resistance, not by surrounding it with an arc. When the oxid-carbon 100 coke reaches the proper temperature the carbid formed becomes liquid.

The principal functions of the hearth are first to retain any oxid-carbon coke or partially formed carbid masses within the zone 110 of high temperature resistance until the carbid reaction is complete, and second, to reflect upon the lower portion of the material in the furnace, the intense heat derived from two sources, viz., the combustion of the 115 carbon monoxid formed by the conversion of oxid and carbon into carbid, and by convection and conduction from the molten carbid falling upon the hearth.

The furnace may be operated by gravity, 120 as can be readily understood from the drawings from the fact that the carbid becomes liquid at the moment of formation. This is an important function, as any carbid formed, immediately flows by gravity over and off 125 the hearth out of the zone of reaction and heat. Therefore, there can be little decomposition or contamination of the carbid.

Any metal compound, oxy-compound, or oxid, may be employed instead of a calcium 130

compound, and the same may be cemented by the action of heat on the hydrocarbon intimately associated therewith.

By producing carbid in accordance with the present invention, the material to be transformed or converted into the product desired may be fed to and delivered from the furnace in a continuous manner without the necessity of heating more material than is necessary for its immediate conversion, or the delivery of more energy or electric current than is necessary to produce the carbid, thereby providing a continuous process from the point of supply to the point of discharge. The material in transit is converted as supplied and the production of carbid consumes just enough energy or electricity for its conversion.

While I have herein described more or less in detail a particular manner of carrying out the process and have indicated generally an apparatus which may be employed, and also have specified as examples certain materials or compounds which may be used, it is to be understood that the invention is not limited to these details other than as specified in the appended claims.

Having now described my invention what I claim is:—

30 1. The continuous process of making a carbid which comprises feeding by gravity to a zone of reaction coked material composed of carbon and a metal oxy-compound, and removing from such zone by gravity the molten carbid substantially as rapidly as produced.

2. The continuous process of making a carbid which comprises feeding to a zone of reaction coked material composed of carbon and a metal oxy-compound, and removing from such zone the molten carbid substantially as rapidly as produced.

3. The process of making a carbid which comprises heating to a point at which carbid is produced a metal oxy-compound impregnated with carbon, and discharging the carbid thus produced from the zone of reaction substantially as rapidly as formed.

4. The process of making carbid which

comprises passing continuously through a heating zone material containing a metal oxy-compound impregnated with rigidly attached carbon in proportion to produce carbid, and discharging the carbid from such zone substantially as rapidly as formed and before decomposition or contamination of the carbid can take place.

5. The process of making carbid which comprises passing continuously through a heating zone material containing a metal oxy-compound impregnated with rigidly attached carbon in proportion to produce carbid, and discharging the carbid from such zone by gravity substantially as rapidly as formed and before decomposition or contamination of the carbid can take place.

6. The process of making a carbid which comprises heating by means of its resistance to the passage of an electric current an intimate coked mixture of metal oxy-compound and carbon, retaining such mixture in the zone of reaction until molten carbid is formed, and removing the molten carbid from such zone by gravity substantially as rapidly as formed.

7. The process of making a carbid which comprises feeding a coked mixture of a metal oxy-compound and carbon to a heat-reaction zone induced and maintained by the passage of electricity through such mixture, maintaining the mixture within such zone until its conversion into carbid is substantially complete, and discharging by gravity the carbid thus produced substantially as rapidly as formed.

8. The process of continuously producing carbid which comprises feeding to a zone of reaction a coked mixture of a metal oxy-compound with cokable carbonaceous material, converting said mixture into molten carbid, and removing the molten carbid by gravity substantially as rapidly as formed.

In testimony whereof, I the said JAMES HENRY REID have hereunto set my hand.

JAMES HENRY REID.

Witnesses:

CHARLES R. WRIGHT, Jr.,  
FLOYD R. CORNWALL.